

## UNITED STATES PATENT OFFICE

2,049,396

PROCESS OF PREPARING COMPOSITIONS  
CONTAINING WOOL GREASE NAPHTHENATESFriedrich Meidert, Frankfort - on - the - Main-  
Griesheim, Germany, assignor to I. G. Farben-  
industrie Aktiengesellschaft, Frankfort-on-the-  
Main, GermanyNo Drawing. Application January 13, 1933,  
Serial No. 651,618. In Germany July 17, 1931

## 5 Claims. (Cl. 134—57)

The present invention relates to a process of preparing products containing a combination of salts of wool grease acids and naphthenic acid or a similar acid formed with one or several of the alkaline earth metals, earth metals or heavy metals.

I have found that new compositions can be obtained by the combination of salts of the wool grease acids with a salt of naphthenic acid or a similar acid. These compositions may be used as driers for varnishes, lacquers and oil paints.

The basis of these compositions is wool grease or wool grease acids which may be used in the crude or purified condition. In comparison with the hitherto known substances containing wool grease the new compositions hereinafter described are of considerable advantage, particularly when they are used as driers. The advantage is derived from the fact that the products obtained according to the present invention contain other acids especially suitable for the preparation of driers, besides wool grease or wool grease acids. As acids of this kind there may be used, in addition to wool grease acids, the acids generally used in the manufacture of driers, such as naphthenic acid, linoleic acid, resin acid or the acids obtainable by the oxidation of paraffin, soft paraffin or petroleum. These acids, herein-after called "additional acids", may likewise be used in the crude or purified condition.

As is known, wool grease can be saponified only in the presence of a considerable excess of alkali. According to a former process the excess of alkali has been removed by neutralizing it with a mineral acid, a valueless waste product being produced. The neutralization by means of sulfuric acid or hydrochloric acid entails the further drawback that, if, for instance, lead salts are used, sparingly soluble sulfates or chlorides are formed in the further course of the process. Large quantities of the said sulfates or chlorides are surrounded by the sticky wool grease drier and can be removed only imperfectly and by a complicated process. All these drawbacks are avoided in the process of the present application. The excess of alkali required for the saponification of wool grease is neutralized, not by a mineral acid, but by an acid forming a valuable constituent of the drier. No valueless waste products are obtained, but there is produced a mixture from alkali soaps of the wool grease acids and the naphthenic acid or another additional acid. The whole mixture can be further worked up so as to produce driers.

According to the present invention the driers may be prepared by first saponifying, while heating, wool grease or wool grease acids with an aqueous solution containing an excess of caustic alkali and then neutralizing the excess of alkali by adding the equivalent quantity of one or more additional acids. The solution of alkali soaps obtained is then caused to yield a precipitate by adding a solution of one or more salts of an alkaline earth metal, an earth metal or a heavy metal. It is also possible to use for the precipitation the solution of a mixture of salts containing several different metals. The salts of the so-called siccative metals, for instance of cobalt, manganese, lead and zinc are of particular importance. The mixture of the salts of wool grease acids and the additional acids thus precipitated is then washed and the washing water is drawn off. The water which still remains in the mixture is eliminated by heating the precipitate until fusing occurs, the residual water being thus evaporated. The fusing point is generally above 130° C. In order to accelerate the fusing process it may be advisable to carry out this process at a reduced pressure.

The stability and solubility of the products thus prepared are further increased by adding to the mixture during the course of the preparation a quantity of about 10 per cent. of solid monocarboxylic acids. As monocarboxylic acids there may be used the solid saturated fatty acids, such as stearic acid. Solid olefinic or aromatic carboxylic acids, the substitution products and derivatives thereof are likewise suitable, for instance crotonic acid, benzoic acid, benzoyl benzoic acid, salicylic acid, anthranilic acid, mandelic acid, cinnamic acid or hippuric acid.

The products of the present invention may also be prepared by heating until fusion occurs a mixture of wool grease or wool grease acids and one or more additional acids together with the oxide or hydroxide of one or more alkaline earth metals, earth metals or heavy metals or with the salts formed by these metals with weak acids which are volatile on heating, such as acetates, carbonates or borates. In this case it is likewise possible to use one metal compound or simultaneously several compounds of different metals. The wool grease and acids applied may be used in the crude or purified condition. The fusing temperature is likewise above 130° C. In order to accelerate the fusing process it may, in this case too, be advisable to carry out this process at a reduced pressure.

The products prepared as described above are completely homogeneous solid resinous substances insoluble in water and alcohol but readily soluble in lacquers, fatty acids, linseed oil and most volatile organic solvents. They are of a tough elastic to brittle nature and constitute very valuable driers for varnishes, lacquers and oil paints.

The following examples serve to illustrate the invention, but they are not intended to limit it thereto, the parts being by weight:

1.—250 parts of wool grease having an acid number of 55 and a saponification number of 125 are saponified, while boiling, with about 6 times the quantity of caustic soda solution required (about 165 parts of NaOH) and the excess of about 145 of NaOH is neutralized with 750 parts of naphthenic acid having an acid number of 265. After having been diluted in a suitable manner the neutral soap solution is mixed, while heating it, with a solution of about 560 parts of crystallized cobalt sulfate. The precipitate of cobalt-wool grease-naphthenate obtained is washed with hot water until the Glauber's salt produced during the precipitation has been completely eliminated. After the final washing water has been drawn off the cobalt-wool grease-naphthenate is fused by heating it in the precipitation vessel at about 130° C. until all of the water is eliminated. The fused mass is then directly run into the containers for delivery.

2.—330 parts of crude or purified wool grease are saponified, while being heated, with a caustic soda solution containing 155 parts of NaOH corresponding to about 4 times the quantity required. The excess of NaOH amounting to about 130 parts is neutralized with 670 parts of naphthenic acid. The soap solution obtained is diluted correspondingly and then mixed, while being heated, first with a solution of 208 parts of lead nitrate and then with a solution of about 380 parts of crystallized cobalt sulfate and the precipitate is washed as described in Example 1. After the final washing water has been drawn off, 4 parts of stearic acid and 4 parts of benzoic acid are added for each 100 parts of cobalt-lead-wool grease-naphthenate and the whole is dehydrated, while stirring at a temperature of about 130° C. until the water contained in the mixture has completely evaporated, this being attained after a short time under reduced pressure.

3.—500 parts of wool grease are saponified by boiling with caustic soda solution containing 140 parts of NaOH, and the excess of 95 parts of NaOH is neutralized with 500 parts of naphthenic acid. The soap solution is diluted and then mixed with 75 parts of triethanolamine; the mixture is then mixed with a solution of 40 parts of crystallized cobalt sulfate, 20 parts of anhydrous manganese sulfate and 140 parts of zinc chloride. The precipitate is washed and dehydrated as described in Examples 1 and 2.

4.—A mixture of 750 parts of wool grease acids and 250 parts of naphthenic acid is heated to about 100° C.; 260 parts of litharge are then slowly added in small portions, while gradually raising the temperature to about 150° C. Stirring is continued at this temperature until the evolution of steam has ceased, the fused mass flows easily and a drop of it placed on a glass plate solidifies to a transparent solid.

5.—A mixture of 500 parts of wool grease and 500 parts of naphthenic acid is heated in a suitable vessel. To the mixture there are added gradually in small portions 300 parts of manga-

nese acetate, while raising the temperature to 200° C. to 210° C. Stirring is continued at this temperature until the acetic acid has nearly completely disappeared. At the same temperature 25 parts of cobaltous hydroxide are added likewise very slowly; stirring is continued until a uniform mass is obtained. The process may be finished at this stage or it may be continued by stirring into the mass which has not been allowed to cool 250 parts of linoleic acid, thus obtaining a completely homogeneous drier extract having a very good drying power.

6.—600 parts of wool grease are saponified by boiling with an aqueous solution of 154 parts of caustic potash and the excess of 84 parts of KOH is neutralized while the mass is hot with 400 parts of linoleic acid. The soap solution obtained is diluted with about 5 to 6 times its weight of hot water and mixed with a solution of 290 parts of manganese sulfate (MnSO<sub>4</sub>). The precipitate thus produced is then washed 3 to 4 times at boiling temperature, the final washing water is drawn off and the water still contained in the precipitate is evaporated while stirring and raising the temperature to 130° C. to 140° C. Towards the end of the fusing process 3 parts of palmitic acid and 6 parts of crotonic acid are added for each 100 parts of the yield. The completely homogeneous fused mass is then run directly into the containers for delivery.

7.—400 parts of crude or purified wool grease are saponified, while boiling, by 100 parts of caustic soda solution, about 3.3 times the quantity required, and the excess, about 70 parts of NaOH, is neutralized with application of heat by means of 600 parts of resin acid. To the neutral soap solution which is diluted there are first added at about 60° C., while stirring, a solution of about 330 parts of lead nitrate. Precipitation is then finished with a solution of about 120 parts of manganese sulfate (MnSO<sub>4</sub>). The precipitate is washed and dehydrated as described in Example 1.

8.—300 parts of wool grease or wool grease acids are saponified, while boiling, by 175 parts of caustic soda solution, about 7 times the quantity required, the excess of 150 parts is neutralized by adding to the hot mass first 350 parts of carboxylic acid obtainable by the oxidation of paraffin and then 350 parts of naphthenic acid. The soap solution obtained is diluted, heated to about 60° C. and mixed with a solution of about 215 parts of zinc chloride and about 115 parts of crystallized cobalt sulfate. As soon as the precipitation is complete, the water is drawn off and the precipitate is washed about 3 to 4 times while hot in the usual manner. During the dehydration 3 parts of salicylic acid and 3 parts of benzoyl benzoic acid are added for each 100 parts of the yield and the whole is maintained at 130° C. to 140° C., while stirring, until a completely homogeneous anhydrous fused mass is obtained. The fused mass is then run into the containers for delivery and solidifies to form a brittle mass. In the following claims there is to be understood by the term "siccative metals" such metals as possess the property of accelerating the drying of the oils, for instance the metals cobalt, manganese, lead and zinc.

I claim:

1. The process which comprises saponifying a compound selected from the group consisting of wool grease and wool grease acids with an aque-

ous solution containing an excess of caustic alkali, neutralizing the excess of caustic alkali with at least one acid selected from the group generally used in the manufacture of driers and 5 consisting of naphthenic acid, linoleic acid, resin acid and the acids obtainable by the oxidation of paraffin, soft paraffin and petroleum, adding a soluble salt of at least one siccative metal 10 washing the precipitate thus produced with water and evaporating the water remaining in the precipitate by heating the precipitate to fusing.

2. The process which comprises saponifying a compound selected from the group consisting of 15 wool grease and wool grease acids with an aqueous solution containing an excess of caustic alkali, neutralizing the excess of caustic alkali with at least one acid selected from the group consisting of naphthenic acid, linoleic acid, resin acid and the acids obtainable by the oxidation 20 of paraffin, soft paraffin and petroleum, adding a soluble salt of a siccative metal washing the precipitate thus produced with water, evaporating the water remaining in the precipitate by heating the precipitate to fusing, and adding a 25 small quantity of a solid monocarboxylic acid during the course of the process.

3. The process which comprises saponifying a compound selected from the group consisting of 30 wool grease and wool grease acids with an aqueous solution containing an excess of caustic alkali, neutralizing the excess of caustic alkali

with naphthenic acid, adding a soluble salt of at least one siccative metal selected from the group consisting of cobalt, manganese, lead and zinc, washing the precipitate thus produced with water, evaporating the water remaining in the precipitate by heating the precipitate to fusing, the fusing process being performed at a reduced pressure and adding a small quantity of a solid monocarboxylic acid during the course of the process.

4. The process which comprises saponifying a compound selected from the group consisting of wool grease and wool grease acids with an aqueous solution containing an excess of caustic alkali, neutralizing the excess of caustic alkali 15 with naphthenic acid, adding a soluble cobalt salt and a soluble manganese salt, washing the precipitate thus produced with water and evaporating the water remaining in the precipitate by heating the precipitate to fusing.

5. The process which comprises saponifying a compound selected from the group consisting of wool grease and wool grease acids with an aqueous solution containing an excess of caustic alkali, neutralizing the excess of caustic alkali with 25 naphthenic acid, adding a soluble lead salt and a soluble manganese salt, washing the precipitate thus produced with water and evaporating the water remaining in the precipitate by heating the precipitate to fusing.

FRIEDRICH MEIDERT.